

## UNITED STATES PATENT OFFICE.

CLARENCE M. CARSON, OF AKRON, OHIO, ASSIGNOR TO THE GOODYEAR TIRE & RUBBER COMPANY, OF AKRON, OHIO, A CORPORATION OF OHIO.

## FABRIC AND METHOD OF TREATING SAME.

No Drawing.

Application filed November 20, 1926. Serial No. 149,796.

My invention relates to the treatment of fabrics and it has for its primary object the provision of a method to render insoluble coatings of impervious material applied thereto.

It is customary practice in the oil industry to provide a flexible fabric container for the purpose of receiving gasoline vapor or moisture, formed in a large gasoline storage tank, and which is evaporated therefrom by solar heat during the day. These containers, which are commonly known as breather bags, are formed of fabric which has been coated with some material to render it impervious to the vapors condensed therein. A mixture of glue and glycerin has been employed for such coatings, but films of this character are objectionable since they are hygroscopic and are quickly deteriorated by atmospheric moisture which condenses upon the outer surface of the bag.

I have discovered that coatings of this general nature may be rendered water-proof by the application of a suitable fixing agent to the film after it has been applied to the fabric. The fabric may be coated, by any desired means, with an impervious mixture, such, for example, as glue and glycerin, which is allowed to dry partially. Thereafter, the surface of the film is sprayed or painted with a solution of a suitable precipitating or tanning agent, such as sodium alum, formaldehyde, or potassium dichromate. The fabric so treated is ready for use when dry.

Preferably, a solution having a relatively low concentration of the tanning agent is desirable; thus, when sodium alum is employed, the concentration should be between three and five percent. It has been found that a higher concentration produces a tendency for the film to shrink and thus allow the glycerin, or other softening agent, to come to the surface, from which it can be dissolved by moisture. This tendency may

be minimized, even with the application of solutions of low concentration, by applying the tanning agent to the coated fabric on a tentering frame similar to those employed in the textile industry.

Various other coating materials may be employed in place of glue glycerin mixtures. Thus, other gasoline resistant materials, such as casein or albumen, may be utilized, and softening agents, such as Turkey red oil or ethylene-glycol, may be employed in place of glycerin. In all cases it is believed that the insolubility results from the hardening by the tanning agent of the glue or other impervious film.

A coated fabric treated in the foregoing manner may be readily manufactured and it is highly resistant to the effects of atmospheric conditions. The material may be handled in the field without the care heretofore employed, because the film has a greater tenacity and is more resistant to cracking, softening, or like defects, which would render the product unsatisfactory for use. Obviously, fabric so treated may be utilized for other purposes than breather bags, as, for example, in the preparation of gasoline-proof hose or the like. The foregoing examples should be regarded, therefore, as illustrative of the principles of the invention, and only such limitations should be imposed as are set forth in the following claim.

## What I claim is:

A method of treating fabrics for breather bags which comprises applying to the fabric a gas-tight coating of proteinous material containing a softening agent, partially drying the coating, stretching the fabric upon a frame, applying a tanning solution thereto and completing the process of drying.

In witness whereof, I have hereunto signed my name.

CLARENCE M. CARSON.